

## UNITED STATES PATENT OFFICE

2,028,029

## WHEEL RIM

Herman Johan van Royen, Horde in  
Westfalia, GermanyNo Drawing. Application August 15, 1932, Serial  
No. 628,959. In Germany August 4, 1931

2 Claims. (Cl. 75—1)

This invention relates to the production from a eutectoid steel of wheel rims, or other articles which are required to offer high resistance to abrasive wear. The invention is the result of experiments which have shown that eutectoid carbon steels containing manganese as a double-carbide former in sufficient amount to lower the carbon content considerably below 0.9%, with a purely lamellar pearlitic structure, exhibit a resistance to abrasion which is not only considerably higher than that of the normalized steels, but also higher than that of eutectoid steels, containing 0.9% of carbon.

It has also transpired that, in general, the resistance to abrasion of lamellar pearlitic eutectoid steels is determined by the content of double-carbide formers in the cementite lamellæ of the pearlite, and that the manganese employed, as double-carbide former, in previous experiments can be wholly or partially replaced by chromium, molybdenum, tungsten and vanadium, with good results. The amount of the other metals, substituted for, or used in association with the manganese, is adjusted so that the carbon content of the eutectoid steel lies between 0.68 and 0.77%, the manganese content being, for example, between 0.40 and 0.85%, the chromium between 0.30 and 0.80%, the tungsten between 0.25 and 0.70%, the molybdenum between 0.22 and 0.65%, and the vanadium between 0.18 and 0.60%.

Further experiments showed unexpectedly that the already high resistance to abrasion of eutectoid steels containing the aforesaid double-carbide formers, can be further increased by raising the silicon content. The silicon content of the hard-wearing eutectoid steels, hitherto produced by applicant, lay between the usual limits of 0.15 to 0.30% for carbon steels, of the same tensile strength, chilled with silicon alone. Slightly increasing the silicon content, for example by a little more than 0.05%, resulted in an unexpectedly high increase in the resistance to abrasion, which can be still further heightened by further addition of silicon. In such case, also, the presence of a purely lamellar pearlitic structure is essential to success since, as is known, a eutectoid steel does not necessarily exhibit a lamellar structure after cooling. Steels, on the contrary, that contain chromium, molybdenum, tungsten and vanadium in addition to manganese, tend to form sorbitic pearlite in normal cooling. Thus the object of this invention is a wheel rim and similar articles offering high resistance to abrasion and exhibiting a purely lamellar pearlitic structure composed of a steel with a carbon content be-

tween about 0.65 and 0.78%, a silicon content between about 0.40 and 0.80% and comprising at least one of the following double carbide formers: manganese between about 0.40 and 0.85%, chromium between about 0.30 and 0.80%, tungsten between about 0.25 and 0.70%, molybdenum between about 0.22 and 0.65%, vanadium between about 0.18 and 0.60%, the balance comprising substantially iron, the sum of said double carbide formers being so proportioned that the composition is eutectoid, the steel having also purely lamellar pearlitic structure in the finished articles.

The following examples represent the composition of steels produced in accordance with the invention:

|    | C %  | Mn % | Si % | Cr % | W %  | Mo % | Va % | 20 |
|----|------|------|------|------|------|------|------|----|
| 1. | 0.70 | 0.51 | 0.78 | 0.49 | —    | —    | —    |    |
| 2. | 0.69 | 0.59 | 0.46 | —    | 0.41 | —    | —    |    |
| 3. | 0.71 | 0.56 | 0.51 | —    | —    | 0.35 | —    |    |
| 4. | 0.75 | 0.45 | 0.54 | —    | —    | —    | 0.34 |    |

The favourable effect of higher silicon contents is evident from the following figures:

Abrasion test in the Mohr & Federhaff tester, under the following conditions:

|                                  |         |    |
|----------------------------------|---------|----|
| Width of abrasive wheels         | 10 mm.  | 30 |
| Pressure applied                 | 100 kg. |    |
| Number of revolutions per minute | 425     |    |
| Slip                             | —1%     |    |
| Hardness of the counter disc     | 500     |    |
| Total number of revolutions      | 250,000 | 35 |

| Chemical composition |      |      |      |                        |
|----------------------|------|------|------|------------------------|
| C %                  | Mn % | Cr % | Si % | Wear (loss),<br>mgrms. |
| 0.67                 | 0.58 | 0.78 | 0.26 | 435                    |
| 0.70                 | 0.58 | 0.43 | 0.30 | 365                    |
| 0.72                 | 0.56 | 0.45 | 0.38 | 230                    |
| 0.69                 | 0.54 | 0.47 | 0.44 | 190                    |
| 0.70                 | 0.51 | 0.49 | 0.78 | 140                    |

The experiments showed that by increasing the silicon content above the ordinary limits, the wear under the specified test conditions is below the minimum, namely 300 mgrms. of that of ordinary hard-wearing steels in the best instances.

In the case of eutectoid steels containing certain percentages of carbon, which will be referred to hereinafter, the experiments also indi-

cated that silicon, in association with double-carbide formers, produces a particularly high resistance to abrasion, and this was not hitherto known. The favourable effect of higher silicon contents on the resistance to abrasion of lamellar pearlitic eutectoid steels containing double-carbides is probably attributable to the modification in the composition of the cementite lamellæ. As is known, the silicon in steel partly passes into the cementite lamellæ of the pearlite. Accordingly, higher percentages of silicon also lower the carbon content of the pearlite. Whether the silicon exists in the cementite, as iron silicide or silicon carbide, or as double- or poly-carbide, has not been definitely established. The fact remains, however, that applicant was able to detect an increase in the resistance to abrasion with increasing silicon content. It is hardly possible to specify the upper limit of the addition of silicon. This will be determined, on the one hand, by the capacity of the cementite for absorbing silicon, and on the other hand by the decomposition of the cementite into carbon (graphite, temper carbon) and ferrite, occurring with high silicon contents and slow rates of cooling. For the production of wheel rims, rails, pinions, spindles, and the like, silicon contents of 0.35 to 0.80% have proved favourable. In this connection, the experiments have shown that, with rising silicon content, the carbon content can be lowered to 0.65%, it being, of course, necessary to adjust the content of double-carbide formers, such as manganese, chromium, tungsten, molybdenum and vanadium, so that a eutectoid steel is obtained in each case.

*Example*

A steel is produced by the bessemer or hearth refining process, or in the electric furnace, having a carbon content of 0.65 to 0.78%. After reduction in the furnace or ladle, ferro-manganese, ferro-chromium, ferro-tungsten or ferro-vanadium is added to the molten metal in such quantities that, after the succeeding addition

of ferro-silicon, to an extent that will give a silicon content of 0.35 to 0.80% in the finished steel, a eutectoid steel is obtained. The steel is then heated and shaped in the usual manner into the specified articles, but the rate of cooling the finished products is regulated, in a simple manner, by insertion in a cooling stove, covering up or packing in piles, so that the finished article exhibits a purely lamellar pearlitic structure.

I claim:

1. Wheel rims and similar articles offering high resistance to abrasion and exhibiting a purely lamellar pearlitic structure, composed of a steel with a carbon content between about 0.65 and 0.78%, a silicon content between about 0.40 and 0.80% and a manganese content between about 0.40 and 0.85% and comprising metal from a group of the double carbide formers: chromium between about 0.30 and 0.80%, tungsten between about 0.25 and 0.70% and molybdenum between about 0.22 and 0.65%, the balance comprising substantially iron, the sum of said double carbide formers being so proportioned that the composition is eutectoid, the steel having also a lamellar pearlitic structure in the finished articles.

2. Wheel rims and similar articles offering high resistance to abrasion and exhibiting a purely lamellar pearlitic structure, composed of a steel with a carbon content between about 0.65 and 0.78%, a silicon content between about 0.40 and 0.80%, a manganese content between about 0.40 and 0.85% and vanadium between about 0.18 and 0.60%, and comprising metal from a group of the double carbide formers: chromium between about 0.30 and 0.80%, tungsten between about 0.25 and 0.70% and molybdenum between about 0.22 and 0.65%, the balance comprising substantially iron, the sum of said double carbide formers being so proportioned that the composition is eutectoid, the steel having also a lamellar pearlitic structure in the finished articles.

HERMAN JOHAN VAN ROYEN.